

L. P. BURROWS.

PROCESS OF TREATING NICKEL ORES AND PRODUCT RESULTING THEREFROM.  
APPLICATION FILED MAY 4, 1920. RENEWED SEPT. 22, 1921.

1,424,711.

Patented Aug. 1, 1922.



### Inventor

*Linus P. Burrows.*

By Spear, Middleton, Donaeson & Hall

Attorneys.

# UNITED STATES PATENT OFFICE.

LINUS PORTER BURROWS, OF ERIE, PENNSYLVANIA; LENAH B. ARCHER EXECUTRIX  
OF SAID L. P. BURROWS, DECEASED.

## PROCESS OF TREATING NICKEL ORES AND PRODUCT RESULTING THEREFROM.

1,424,711.

Specification of Letters Patent.

Patented Aug. 1, 1922.

Continuation of application Serial No. 335,107, filed November 1, 1919, which in turn is continuation of Serial No. 44,310, filed August 7, 1915. This application filed May 4, 1920, Serial No. 378,895. Renewed September 22, 1921. Serial No. 502,549.

To all whom it may concern:

Be it known that I, LINUS PORTER BURROWS, a citizen of the United States, and resident of Erie, Pennsylvania, have invented certain new and useful Improvements in Processes of Treating Nickel Ores and Product Resulting Therefrom, of which the following is a specification, the same being a continuation of application filed August 7th, 10 1915, and serially numbered 44,310.

This discovery and invention relates to an alloy for use in steel making that is made from nickel ores, and it includes the refining of such ores as well as related ores, it being 15 specially adapted to the Sudbury nickel ores and it consists in the treatment of the ore as hereinafter described.

The process may be carried out in any suitable apparatus and I have illustrated 20 one embodiment of apparatus which may be used for this purpose, although it will be understood that this is illustrative only and that any other apparatus which would enable the various steps of the process to be 25 carried on in the manner stated could be used.

The drawing shows a sectional elevation of the apparatus.

The apparatus comprises an expansion, 30 radiation and precipitation chamber A, a digester B, and a plurality of precipitating chambers C only one of which is shown. The digester B includes a treating chamber E in which the material is treated, and for 35 convenience in agitating the material the treating chamber is constructed in the form of a rotatable drum having hollow side trunnions 10 and 11 secured to the ends 12 and 13 of the drum.

Suitable means are provided for heating 40 the material in the drum, and in the embodiment illustrated I have surrounded the treating chamber with a furnace or heating chamber F constructed with a suitable sheet metal shell 14 lined with firebrick or other heat resisting material 15.

The heating may be accomplished by any 45 of the well known means of a gas burner supplied with a gas supply pipe 17.

The air for combustion of the gas may

pass in through the opening 18 and the products of combustion flow out through the opening 19.

The turning of the treating chamber is accomplished by convenient means, such as the 55 gear 20 mounted on the trunnion 11 and driven from a pinion 21 on the counter-shaft 22, which countershaft is supported by suitable bearings 23 and 24 and driven from a pulley 25. The trunnions 10 and 11 60 are supported by bearings 26 and 27.

The expansion, radiation and precipitating chamber A is in the form of a cylindrical container of considerable size, in which the steam is adapted to suddenly expand 65 from substantially the center of the container, being introduced to the center by a pipe 40 which extends through the side of the chamber. On the top of the chamber is 70 a dome 41 from which the expanded and dried steam passes into a delivery pipe 42.

A weighted pop-valve 43 leads from the pipe 8 into the atmosphere and serves to maintain a substantially uniform pressure in the said pipe. The pipe 42 also contains 75 a control valve 44.

The water of precipitation is removed by a suitable valved outlet 45 at the bottom of the chamber controlled by a ball float 46 which causes the water to flow off as soon as 80 it rises to any considerable height in the bottom of the chamber. A manhole 47 may be provided for the removal of any sludge, normally closed by a door 48.

The steam which forms the base of the 85 gaseous reagent may be produced in any convenient way. After the process is started it may be produced by a heat radiating from the furnace F and accordingly a heating coil H is shown embedded in the walls 90 of the furnace applied by a pipe 51 leading from a suitable water source.

From coil H a pipe 52 leads to the expansion and radiation chamber A. From the expansion and radiation chamber the result- 95 ant gas passes by the pipe 42 and a pipe 53 to suitable coils 1 embedded in the walls there- of whereby the gas is superheated to a high temperature. When superheated, the result- ant gaseous product passes by the pipe 54 100

to the valved injecting nozzle 55, which projects through the hollow trunnion 10 having a gas tight joint therewith. The gaseous product is discharged through the nozzle into the chamber E to deoxidize the material therein. A suitable pressure gauge 56 may be provided to indicate the pressure at this point and the flow may be controlled by a suitable valve 57.

10 The excess gaseous products in the chamber E pass through the hollow conduit 60 leading to the side of the first precipitating chamber C.

15 A plurality of similar precipitation chambers will be provided connected in series.

It will be seen that in the ordinary operation steam under moderate pressure will be delivered from the pipe H. This passes into the expanding, precipitating and radiating chamber A where it is subjected to

20 sudden expansion with diminution of pressure under such conditions as to prevent any material condensation and to allow the watery particles that are held in suspension

25 in the steam to separate from the steam by gravity or otherwise and become precipitated at the bottom of the chamber whence they pass through the outlet 45. The steam thus deprived of its watery constituents and hav-

30 ing the major portion of the oxygen contained in it radiated through the walls of the cylinder now passes from the dome 41, into the pipes 42 and 53, as a gaseous product, then through the reheating coils 2

35 where any remaining oxygen is separated from the said gaseous product, part of which is discharged into the digester E and part of which may be fed into the burner

16 to be burnt with the gaseous fuel therein.

40 The gaseous product is the same as described in the United States Patent No. 680,313, granted to me August 13th, 1901.

The nickel ore to be treated is crushed to about 40 mesh and then introduced into 45 the rotatable drum provided with means for heating the drum to red heat with conduits for conducting gas to and from the drum. The ore used may have a far lower metal content than anything heretofore capable of 50 commercial use. My treatment recovers all the metallic substance in whatever form it appears and largely in excess of any process now known or practiced. Nitrous or chlorine substances may be added to the ore.

55 After the drum has been charged with ore, it is sealed to the air, the burners under it lighted, the drum slowly revolved, and the gas made in accordance with my Patent 680,313 let into the drum resulting in the instantane-

60ous absorption of the oxygen in the air contained in the drum and the absorption of the oxygen in the ore immediately following. From five to six hours the drum is rotated and kept at red heat

65 with a constant inflow of the gas and an out-

flow of gas through the outlet from the drum and through a series of precipitating chambers.

The contents of the drum are then removed and smelted in a crucible or otherwise, causing the metalliferous substances to separate from the silicious substances, the latter taking the form of a glassy slag. The purified metallic product is then broken up by a hammer or the like into lumps approximating the size of furnace coal. These lumps are exposed to the atmosphere for a period of from 12 to 24 hours, depending upon their size, resulting in a perfect disintegration of the lumps into a very fine powder. The powder can then be used as an alloy. The powder is about one half soluble in sulphuric or nitric acid. It is particularly pointed out that no roasting of the ore takes place.

This powder, I discovered by actual test in melting it with steel or iron scraps by the proportion of from 3 percent to 6 percent, produces a very fine cast metal corresponding in atomic structure to brass and other non-magnetic alloyed metals, but it has much greater rigidity and tensile strength. I also discovered that by the use of this powder the ordinary expansion of steel or iron between red and cold heat has 95 been reduced to a minimum. It also corresponds with brass in not being forgeable when heated. The powder is of a brownish-black cast also impalpable, about the condition of flour and is exceedingly useful as 100 an alloy in iron and steel and particularly in pig iron and steel scrap in producing metal castings.

The use of this powder also clarifies the mixture to a remarkable degree. 105

It is, of course, intended that all matter contained in the accompanying specification and drawings shall be interpreted as illustrative and not in a limiting sense.

What I claim as my invention is: 110  
1. The process herein described consisting in first suddenly expanding steam, then separating the steam without condensation from any water held in suspension, then heating the resultant gaseous product and then subjecting crushed nickel ore in a closed chamber to the action of the gaseous product for approximately five hours at red heat.

2. The hereinbefore described process consisting in first suddenly expanding steam, then separating the steam without condensation from any water held in suspension, heating the resultant gaseous product, and then subjecting crushed nickel ore to the action of the gaseous product for approximately five hours at red heat; subjecting the refined nickel ore to a smelting process to separate the silicious matter from the metalliferous matter; then breaking up the me- 130

tallic product and exposing it to the atmosphere, whereby a complete disintegration of the material takes place resulting in a very fine powder.

5 3. A product made from nickel ore comprising a very fine brownish-black air disintegrated powder, approximately one-half of

said powder being soluble in either sulphuric or nitric acid.

4. A metallic product made from nickel ore comprising an air disintegrated powder.

In testimony whereon I affix my signature this 30th day of April 1920.

LINUS PORTER BURROWS.